

1

2,894,890

## JACKETING URANIUM

Henry A. Saller and John R. Keeler, Columbus, Ohio, assignors to the United States of America as represented by the United States Atomic Energy Commission

No Drawing. Application July 20, 1949  
Serial No. 105,907

11 Claims. (Cl. 204—193.2)

This invention deals with the plating of uranium, and in particular with the bonding, to uranium, of plates of iron, or cobalt, or nickel, or metals based thereon or alloys thereof.

For most uses uranium has to be protected against corrosion, and thus it is enclosed in a metal container or "canned"; for instance  $U^{235}$ , for the generation of power by fission, is used in the form of blankets, rods, slugs, or tubes which are enclosed in a jacket of these above-mentioned metals and preferably of nickel or stainless steel. For all purposes it is necessary that the jacket is bonded to the uranium and that the bond is reliable, durable and resistant to the elevated temperatures prevalent during operation of the power pile.

It is thus an object of this invention to provide a bond between uranium and metals of the iron group of the periodic system of elements which has a long service life even at elevated temperatures.

It is another object of this invention to provide a bond between uranium and metals of the iron group which has a high thermal conductivity.

It is still another object of this invention to provide a bond between uranium and metals of the iron group which is free from cracks and voids and remains in that condition during use at elevated temperatures.

It is also an object of this invention to provide a bond between uranium and metals of the iron group which is characterized by a high degree of homogeneity.

These and other objects are accomplished by coating both surfaces to be joined, namely, the uranium surface and the surface of the jacket or the coating, with silver, amalgamating or alloying these silver coatings with mercury or indium, assembling the uranium core and the metal jacket, exerting pressure, e.g., at room temperature, on this assembly and thereby reducing the area of the assembly, and finally heating the assembly in order to homogenize the silver alloys by diffusion.

The silver layer has been applied to the uranium and the jacket by hot dipping as well as by electro-deposition. While both methods yield satisfactory coatings, the latter method is preferred because no oxide formation or oxygen absorption takes place in that case.

The thickness of the silver layers may be varied considerably and is advantageously adjusted to the dimensions and the use of the final article. For plating the inside of the jacket, for instance in the case of a nickel jacket, a thickness ranging from 0.0001 to 0.001" has been found satisfactory, while for the silver layer on the uranium article a thickness of 0.002 to 0.005" was preferred. In deciding on the thickness of these coatings, it is well to allow for a clearance of from 0.015 to 0.01" between the jacket and the uranium core.

Prior to the amalgamating or alloying step, it is advantageous, though not obligatory, to clean the surfaces. Carbon tetrachloride has been found suitable for this purpose. Thereafter the silver coatings are alloyed with mercury or indium in any conventional manner, and the

2

uranium and jacket are then assembled. The unit is then pushed through a die, for instance, in the case of cylindrically shaped articles, through a wire-drawing die whereby the area is reduced; an area reduction of from

5 to 10% with regard to the actual metal present suffices. The load applied during extrusion is dependent on the dimension of the article and other factors which are known to those skilled in the art. In most cases a pressure of about 325 p.s.i. has been found suitable.

10 The diffusion heating is preferably carried out for from two to four hours at a temperature between 350 and 450° C.; heating for four hours at 450° C. yielded the best results.

In a number of cases where 0.002" thick silver layers 15 had been applied to both the uranium and the jacket, the composition of the alloys formed was determined after completed bonding and heat treatment. The alloys formed were found to vary between 0.059 to 0.091 gram of mercury and from 0.418 to 0.560 gram of silver per 20 inch of the final rod; the mercury content of the alloys varied from 12.5 to 16.5%.

For silver coating the uranium cores, the following procedure was found advantageous:

The uranium core was first anodically cleaned in a 25 solution containing six ounces per gallon of "Anodex," which is an alkaline compound yielding a pH of 12 with ten ounces per gallon of water. The temperature of the bath was 180° F. and the current density was 75 a.s.f. Thereafter the core was rinsed with water and immersed

30 for three minutes into a 35% solution of nitric acid at room temperature. The excess of nitric acid was then removed from the uranium by rinsing it with hot water and then the core was anodically pickled in a bath containing 50% by weight of phosphoric acid and 20 cc. per

35 liter of 37% hydrochloric acid with the bath at room temperature and a current density of 45 a.s.f. Thereafter the core was again rinsed with cold water and then immersed for five minutes in a 35% nitric acid solution. After another rinse with hot water, the core was ready for

40 the silver coating. This was obtained by electrodeposition at 113° F. from a bath containing 75 g./l. of  $AgCN$ , 122 g./l. of  $KCN$ , and 22.5 g./l. of  $K_2CO_3$ ; the pH of this electrolyte had been adjusted to a value of 13 by means of KOH. The current density used was 25 a.s.f.; 45 the time of electrolysis depended on the thickness desired of the silver layer.

The nickel jacket was prepared and coated in a similar manner. It was first cleaned with trichloroethylene and then brushed with a mixture of pumice and a solution of 50 "Nacconol," which is a wetting agent consisting essentially of the sodium salt of a sulfonated alkyl aromatic. Then the nickel jacket was anodically cleaned with "Anodex" of a concentration of six ounces per gallon of water; a current density of 75 a.s.f. was used for three

55 minutes. Thereafter the nickel jacket was electropolished by applying a current density of 200 a.s.f. to a bath composed of 15% sulfuric acid, 63% phosphoric acid and 22% water, at a temperature of 120° F. Thereafter the polished nickel jacket was treated in a bath containing

60 250 g./l. of  $NiSO_4 \cdot 6H_2O$  and 50 g./l. of  $H_2SO_4$  at room temperature with a current density of 150 a.s.f., first anodically for ten seconds and then cathodically for one minute. The next bath used consisted of 7.5 g./l. of  $AgCN$  and 75 g./l. of  $KCN$  and was at room temperature;

65 the jacket was immersed for two minutes while a current density of 5 a.s.f. was applied. Finally the silver coating proper was carried out using an electrolyte composed identically with that used for silver coating the uranium, also at 113° F., but using a current density of 15 a.s.f.

70 It will be understood that the above is merely one possibility of carrying out the silver plating steps and that other conventional ways may be used instead. How-

ever, not all of the preparatory steps described are necessary, nor is the silver plating per se being considered novel and part of the invention. The invention rather lies in the further bonding treatment of the silver-coated members.

The bonds made by the process of the invention show great durability. Heating to temperatures up to 600° C. for about 150 hours in an argon atmosphere did not impair at all the bond obtained. Only a very slight degree of diffusion occurred, when the bonded article was heated at 700° C. for 125 hours. Likewise, cycling between temperatures of 100° C. and 550° C. as often as 60 times did not bring about any harmful effect on the quality of the bond.

Equally satisfactory results were obtained with jackets consisting of the metals set forth above but using indium as the alloying metal instead of mercury.

It will be understood that the invention is not intended to be limited to the details given in the specification, since modifications may be made within the scope of the appended claims.

What is claimed is:

1. A method of securely bonding to uranium a plate based on at least one metal selected from the group consisting of iron, cobalt, nickel and alloys thereof, comprising coating both the surfaces to be bonded with silver, alloying said silver coatings with a metal selected from the group consisting of mercury and indium, assembling said plate and said uranium member, exerting pressure onto the assembly obtained, and heating said assembly whereby the bonding layers are homogenized.
2. The process of claim 1 wherein the silver coating is obtained by electrodeposition.
3. The process of claim 1 wherein the silver coating is obtained by immersing into molten silver.
4. The process of claim 1 wherein the pressure applied

onto the assembly is used so as to reduce the area of said assembly by from 5 to 10% with regard to the actual metal present.

5. The process of claim 1 wherein the final homogenizing heating is carried out for from 2 to 4 hours at from 350 to 450° C.

6. The process of claim 1 wherein the final homogenizing heating is carried out for about 4 hours at approximately 450° C.

7. A shaped article comprising a uranium core, a sheath therearound consisting of a material based on at least one metal selected from the group consisting of iron, cobalt, nickel and alloys thereof, and an intermediate metallic bonding layer consisting substantially of a silver base metal.

8. The article of claim 7 wherein the sheath consists of a nickel metal.

9. The article of claim 7 wherein the sheath consists of stainless steel.

10. The article of claim 7 wherein the bond layer consists of a silver amalgam.

11. The article of claim 7 wherein the bond layer consists of a silver-indium alloy.

#### References Cited in the file of this patent

#### UNITED STATES PATENTS

|           |                  |                |
|-----------|------------------|----------------|
| 1,700,454 | Schumacher       | Jan. 29, 1929  |
| 2,094,483 | Weder            | Sept. 28, 1937 |
| 2,157,933 | Hensel et al.    | May 9, 1939    |
| 2,387,903 | Hensel           | Oct. 30, 1945  |
| 2,476,644 | Wallausen et al. | July 19, 1949  |
| 2,479,882 | Wallausen et al. | Aug. 23, 1949  |
| 861,390   | France           | Oct. 28, 1940  |

#### FOREIGN PATENTS